

May 15, 1956

R. A. GRANGE ET AL  
METHOD OF RESTORING HARDENABILITY  
OF BORON-CONTAINING STEEL  
Filed Oct. 13, 1954

2,745,776

FIG.1.



FIG.2



Inventors:

RAYMOND A. GRANGE and  
ERNEST C. TURNER,

by: Donald G. Dalton  
their Attorney.

**1**

2,745,776

**METHOD OF RESTORING HARDENABILITY OF BORON-CONTAINING STEEL**

Raymond A. Grange, Livingston, N. J., and Ernest C. Turner, Library, Pa., assignors to United States Steel Corporation, a corporation of New Jersey

Application October 13, 1954, Serial No. 461,962

2 Claims. (Cl. 148—21.55)

This invention relates to a method of obtaining the full hardenability effect of boron in boron-containing steels and more particularly to a method of restoring the full hardenability effect of boron in steels that have been austenitized or carburized at temperatures above about 1650° F.

The effect of a minute percentage of boron in greatly increasing the hardenability of many grades of steel has been known for many years. However, certain observers have noted that this hardenability effect is greatly diminished when such steels are austenitized at temperatures in the vicinity of 1650° F. or higher. This is contrary to the effect obtained in nonboron-containing steels since hardenability is increased in most such steels by grain coarsening at high temperatures. This unique effect of boron of lowering hardenability upon austenitizing is particularly undesirable in carburizing steels since in steel parts used in the carburized condition, it is common practice to quench directly from the carburizing furnace or pot in which the steel has been held at an austenitizing temperature for several hours at a temperature sufficiently high to diminish greatly the effect of boron.

It is accordingly an object of the present invention to provide a treatment for boron-containing steels which will restore the full hardenability thereto after such steels have been austenitized at sufficiently high temperatures to diminish the effect of boron on hardenability.

We have discovered that this object can be attained and substantially the full effect of boron restored by holding the steel at or slow cooling to the  $Ar_3$  temperature or slightly above. For most steels of the type involved, this will be a temperature between 1500 and 1600° F. after austenitizing and prior to quenching. Holding at the  $Ar_3$  temperature for sufficient time to equalize the temperature following rapid cooling will suffice. At this temperature some of the boron dissolved in the austenite by the high austenitizing temperature precipitates and thus reduces the amount of boron dissolved in austenite to the optimum amount for good hardenability. Temperatures below the  $Ar_3$  must be avoided because of the tendency for ferrite to form. Ordinarily this heat treatment would

**2**

involve treating the steel after austenitizing and just before quenching by either cooling to the  $Ar_3$  temperature in the austenitizing furnace or by transferring the austenitized steel to a second furnace maintained at a temperature at the  $Ar_3$  temperature and holding it there for sufficient time to equalize the temperature at or just above the  $Ar_3$  temperature.

The attached Figures 1 and 2 of the drawing are illustrative of the teachings of our invention. Each of the graphs show end-quench hardenability data obtained after treating SAE-86B20 hot-rolled steel bars of 1½ inch diameter. The steel contained .18% carbon, .83% manganese, .49% nickel, .49% chromium, .19% molybdenum and .0013% boron. Figure 1 shows the reduction in hardenability by holding at 17 hours for the temperatures indicated. Thus line 1 shows the effect of holding at 1650° F., line 2 at 1700° F. and line 3 at 1750° F. In Figure 2, the result of following the teaching of the invention by holding at a lower temperature is clearly shown. In this figure, line 1 indicates the end-quench hardenability of the bars after heating at 1700° F. for 20 minutes, line 3 after heating at 1750° F. for 17 hours and line 2 the effect of holding bars, previously heated at 1750° F. for 17 hours, at 1550° F., i. e. the  $Ar_3$  temperature for one hour prior to quenching. This shows that substantially the full hardenability effect of the boron is restored by holding at the lower temperature prior to quenching.

This application is a continuation-in-part of our co-pending application Serial No. 235,232, filed July 5, 1951, now abandoned.

While we have shown a specific example of our invention, it will be understood that this example is merely for the purpose of illustration and description and that various other forms may be devised within the scope of our invention, as defined in the appended claims.

We claim:

1. A method of restoring the hardenability effect of boron in boron-containing steel which has been diminished by austenitizing the steel at a temperature above 1650° F. comprising holding the austenitized steel prior to quenching at the  $Ar_3$  temperature for sufficient time to equalize the temperature of the steel at said temperature and precipitate boron dissolved in the austenite by said austenitizing.
2. A method of obtaining the full hardenability effect of boron in boron-containing carburized steel comprising carburizing the steel at a temperature in excess of 1650° F., equalizing the temperature of the carburized steel at the  $Ar_3$  temperature to precipitate excess boron dissolved in the austenite by said austenitizing and then quenching said steel.

**References Cited in the file of this patent**

"Metals Handbook," 1948 ed., pages 684 and 685.